

Feb. 20, 1951

J. H. FRIEDMAN  
METHOD OF MAKING NUTS

2,542,023

Filed Aug. 3, 1944

2 Sheets-Sheet 1

Fig. 1a



Fig. 1

Fig. 2a



Fig. 2

Fig. 3a



Fig. 3



Fig. 4a



Fig. 4

INVENTOR.  
JOHN H. FRIEDMAN

BY

Rickey & Watto.  
ATTORNEYS

Feb. 20, 1951

J. H. FRIEDMAN  
METHOD OF MAKING NUTS

2,542,023

Filed Aug. 3, 1944

2 Sheets-Sheet 2



Fig. 6



INVENTOR.  
JOHN H. FRIEDMAN

BY

Rickey & Watts.  
ATTORNEYS

## UNITED STATES PATENT OFFICE

2,542,023

## METHOD OF MAKING NUTS

John H. Friedman, Tiffin, Ohio, assignor to The National Machinery Company, Tiffin, Ohio, a corporation of Ohio

Application August 3, 1944, Serial No. 547,849

31 Claims. (Cl. 10—86)

1

This invention relates to a process for making nuts and similar articles.

In prior efforts to produce nuts and similar polygonal articles by cold forging the articles from wire or rod stock great difficulty has been encountered in attempting to make the metal flow into the desired polygonal shape so as to produce sharp, well filled corners. If excessive pressures or excessive metal flow are resorted to, the dies and tools are rapidly destroyed and the metal in the articles is excessively work-hardened, tending to cause such excessive hardness and brittleness that the articles cannot be machined, as required, for example, in the tapping of nut blanks.

I have discovered that this and other difficulties and problems in the making of such articles can be overcome by shaping a blank with respect to a die to cause the blank itself to act as a force multiplier, so that the desired metal flow is obtained without applying excessive pressures to the blank.

Another feature of the present invention is the arranging of the metal in a blank with respect to a die so that the necessary pressure per unit area is applied to small areas of the blank requiring the greatest flow with a substantially smaller unit pressure applied to the face of the blank.

In one embodiment of the present invention such force multiplication and increased unit pressures are obtained in somewhat different ways in each of two separate steps. In each step a blank is upset into a die which has at least a portion of its end face arranged at a greater angle with the adjacent side wall of the die than the corresponding angle between the end face and side wall of the blank. Thus when the blank is upset into the die the blank acts as a force multiplier and applies a greater unit pressure at the corners between the end face and the side wall of the die than the average unit pressure applied to the front face of the blank.

In the preferred embodiment, this action is obtained in one step by upsetting a blank which has side walls substantially perpendicular to its end face into a die with a generally concave bottom, the side walls of which form an obtuse angle with the adjacent portions of the bottom wall of the die. The blank is upset by means of a punch having a generally convex face, producing a dished, or concavo-convex blank. In the upsetting action the side walls tend to retain their original angular relationship with the faces of the blank, so that the metal is pressed

2

radially outward with great force in the region of the corner between the side walls and the bottom face of the die by a leverage action within the blank itself. All corners adjacent the convex face of the blank are thereby filled completely and sharply.

In the next step in the preferred embodiment, the blank produced by the foregoing operation has its concave face engaged with the bottom 10 of a die recess which has side walls substantially perpendicular thereto. The blank is again upset, and the corners adjacent the concave face are forced strongly outward by a toggle or leverage action. By the combination of these two 15 actions the corners of a polygonal blank are filled completely and sharply with the application to the blank of only relatively low pressures.

Another feature of the present invention is the 20 punching of an axial hole through the blank without distorting the exterior surface or causing the blank to freeze in a die. This is accomplished, in the preferred embodiment, by confining the side walls of the blank exteriorly 25 through a portion only of their height adjacent one face of the blank, and forcing a punch into the blank from the other face. The metal of the blank is thereby permitted to spring outwardly during the punching, while permanent deformation is prevented by the confining of the one face and adjacent portions of the side walls. The limited area of engagement between the blank and the die permits the blank to free itself readily when the punch is retracted.

35 Other objects and advantages of the invention will appear from the following detailed description of a preferred embodiment of the method and apparatus for carrying out the same.

In the accompanying drawings:

40 Fig. 1 is a sectional view with parts in elevation taken through the stock feed station of a machine arranged to carry out the present invention;

45 Fig. 1—*a* is an elevation of a cut-off blank; Fig. 2 is a sectional view, with parts in elevation, through the next station of the machine; Fig. 2—*a* is an elevation of the blank produced by the die shown in Fig. 2;

50 Fig. 3 is a sectional view, similar to Figs. 1 and 2, through the dies constituting the next station of the machine;

Fig. 3—*a* illustrates in cross section and in elevation the blank produced by the dies shown in Fig. 3;

55 Fig. 4 is a sectional view through the next

station of the machine, showing the step of dishing the blank;

Fig. 4-a illustrates in cross section and in elevation the dished blank produced by the tools shown in Fig. 4;

Fig. 5 is a section through the next station of the machine, showing the step of again flattening the dished blank;

Fig. 5-a illustrates in section and in elevation the blank produced by the tools shown in Fig. 5;

Fig. 6 is a section through the punching station of the machine, showing the parts after completion of a punching operation;

Fig. 6-a illustrates in cross section and in elevation the punched blank; and

Fig. 7 shows the stripping of the blank from the punch on the retracting stroke of the punching tools.

The dies and tools shown may be mounted in a multiple station transfer header with all of the dies mounted in the bed frame and the cooperating tools carried by a reciprocating header slide, and with a transfer mechanism to carry the blanks from each station to the next and to turn the blank over between each two successive operations. Such a machine is disclosed and claimed in the patent to Frayer No. 2,100,028. The invention, however, is not limited to such a machine, as the method of this invention may be carried out in a plurality of separate machines, by hand, or in one or more multiple station headers of other types, such as the machine disclosed and claimed in the patent to Clouse No. 2,026,823. Similarly, the novel dies and tools of this invention may be mounted in any desired machine or machines, or may be manipulated by hand. For maximum economy of operation, however, it is preferred to utilize a machine which performs all of the operations without intermediate handling, and for simplicity in the mounting of the dies and tools the machine of the aforesaid Frayer Patent No. 2,100,028 is preferred.

Any suitable means may be employed to supply blanks to the process. The cut-off mechanism illustrated in Figs. 1 and 2 is of the type disclosed and claimed in my U. S. Patent No. 2,396,995, granted March 19, 1946, on co-pending application Serial No. 547,886, filed August 3, 1944, a continuation in part of my application Serial No. 423,900, filed December 22, 1941, which has since become abandoned. The bed frame 10 of the machine is provided with an opening 11 through which wire or rod stock S is fed by any suitable feeding means (not shown). A shear arm 13 carrying a bushing or sleeve 14 arranged to surround the stock S is mounted for reciprocation along the face 15 of the bed frame 10. A plunger 16 having a head 17 is slidably mounted in and carried by the bushing 14.

When the bushing 14 is in alignment with the hole 11 the stock S is fed forwardly until the head 17 of the plunger 16 engages a stock gauge 18 which is adjusted to permit the desired length of stock to be entered into the bushing 14. Thereupon the shear arm 13 is moved across the face 15 of the bed frame 10 in the direction of the arrow shown in Fig. 1, so that the edges of the opening 11 in the bed frame 10 and the adjacent edges of the bushing 14 cooperate to shear a blank 19 from the stock S.

The shear arm 13 continues to move until the bushing 14 is brought into alignment with the opening in a die 20 mounted in the bed frame 10 as illustrated in Fig. 2. During this move-

ment of the shear arm 13 the head 17 of the plunger 16 slides across the stock gauge 18, the plunger 16 remaining in position in the bushing 14.

When the bushing 14 is aligned with the opening in the die 20 the motion of the shear arm 13 ceases and a punch 21 mounted in the reciprocating header slide 22 advances against the head 17 of the plunger 16. The motion of the punch 21 continues until the plunger 16 forces the blank 19 out of the bushing 14 and upsets the same into the opening in the die 20. The position of the parts at the end of the forward travel of the punch 21 is illustrated in Fig. 2.

In the present process the die 20 is preferably provided with a conical bottom wall 23 surrounding a knock-out pin 24, so that the blank 25, formed in the die 20 has a conical or chamfered surface 26, as shown in Fig. 2-a. The upsetting of the blank 19 into the die 20 to form the blank 25 serves to size the blank by pressing it into close contact with the wall of the opening in the die 20, to remove any irregularities of the end faces produced by the shearing action, and eliminate any non-uniformities in cross sectional shape which may have existed in the stock S. A spring 27 preferably surrounds the plunger 16 and engages the head 17 and the adjacent end of the bushing 14 when the punch 21 has reached the limit of its forward movement as shown in Fig. 2. As the punch 21 is retracted the spring 27 withdraws the end of the plunger 16 from the opening in the die 20 and the shear arm 13 thereupon returns to its position in alignment with the stock feed opening 11, as illustrated in Fig. 1. Thereupon the knock-out pin 24 ejects the blank 25 from the die 20, where it is seized by the transfer mechanism and delivered to the next die.

In the illustrated embodiment the next station of the machine embodies a die 28 mounted in the bed frame 10 and having an opening of hexagonal or other polygonal cross section. The bottom of the die opening is formed by a hexagonal knock-out pin 29 slidably fitting within the die opening. The blank 25 is turned over while being transferred from the die 20 to the die 28, as disclosed in the aforesaid patent to Frayer No. 2,100,028.

A punch 30 mounted in the reciprocating header slide 22 is arranged to engage the blank 25 after the same has been turned over and positioned in front of the die 28 by the transfer mechanism. After engaging the blank 25 the punch 30 forces the same into the die 28 and upsets the blank against the end of the knock-out pin 29 so as to partially form the blank to the polygonal cross section of the opening in the die 28. The punch 30 is arranged to apply only a relatively light upsetting pressure to the blank, so as to shorten the same and flatten the metal into contact with the flat sides of the hexagon defined by the die 28, without attempting to flow the metal to fill up the corners of the hexagon. This operation produces the blank 31, shown in Fig. 3-a, having partially formed flat areas 32 corresponding to the flats of the hexagon defined by the opening in the die 28. As the punch 30 recedes, the knock-out pin 29 ejects the blank 31 from the die 28 into the transfer mechanism to be carried to the next station of the machine. The blank is again turned over and transferred to a position in front of a die 33 carried in the bed frame 10, illustrated in Fig. 4. The die 33 has an opening with a hexagonal cross sectional

shape corresponding to the shape of the opening in the die 28. The bottom of the opening in the die 33 is formed by a wall 34 in the die having a generally conical shape and disposed at an obtuse angle to the side walls 35 of the opening. A knock-out pin 36 forms the center of the bottom wall 34 and is provided at its end with a nose 37 arranged to indent the center of the blank.

A punch 38 carried by the reciprocating header slide 22 is arranged to cooperate with the die 33. The face of the punch 38 is provided with a nose 39 surrounded by a substantially conical surface 40 which is arranged substantially parallel to the conical bottom wall 34 in the die 33.

When the blank 31 is positioned in front of the die 33 it is engaged by the punch 38 and forced into the opening in the die 33. The metal of the blank is upset into the die 33 and by reason of the substantially parallel conical faces 34 and 40 on the die and the punch the blank as a whole is dished. At the same time the nose 37 on the knock-out pin 36 and the nose 39 on the punch indent the blank centrally in the zone that is ultimately to be punched out to form the hole. The bending of the blank in the dishing action tends to force the metal of the blank adjacent the bottom face 34 of the die radially outward, since the bottom face of the blank tends to retain its original substantially perpendicular relation to the side walls of the blank. This radial force drives the metal strongly into the corners between the flat surfaces of the hexagon defined by the opening in the die 33, filling up these corners complete and sharply. This action is assisted by the nose 37 on the knock-out pin 36 which enters the adjacent end face of the blank and tends to spread the same radially outward. This step produces the dished, or concavo-convex, blank 41, illustrated in Fig. 4-a, having indentations 42 and 43 formed by the noses 37 and 39, and having well filled corners 44 adjacent the convex end face 45. At the completion of the operation illustrated in Fig. 4 the punch 38 is retracted and the blank 41 is ejected by the knock-out pin 36 into the transfer mechanism.

The blank 41 is then turned over and transferred into alignment with the die 46 mounted in the bed frame 10. This die is formed with an opening having a hexagonal cross section corresponding to the openings in the dies 33 and 28, and has a bottom wall 47 substantially perpendicular to the side walls 48 of the die opening. For making the usual type of nut having a washer face, the bottom wall 47 may be formed with a step 49. The blank 41 is upset into the die 46 by a punch 50 carried by the reciprocating header slide 22. The punch 50 has a substantially flat end face 51 surrounding a central nose 52, the face 51 being substantially perpendicular to the side walls 48 of the die opening. As the blank 41 is forced into the opening in the die 46 by the punch 50 the blank as a whole is bent to remove the concavo-convex shape imparted to it in the previous operation.

The concave face of the blank 41 is disposed adjacent the bottom wall 47 of the die 46, so that as the blank is flattened out by pressure of the punch against the convex face 45 the metal of the blank adjacent the bottom wall 47 of the die is forced radially outward. This action forces the metal strongly into the corners between the flats of the hexagon defined by the die opening so as to fill up these corners completely and sharply. The knock-out pin 53 is formed with a nose 54 which enters the recess 43 in the blank

41, while the nose 52 on the punch 50 enters the recess 42 in the blank. The flat surface 51 of the punch 50 flattens the convex face 45 of the blank 41. In the type of nut illustrated, a slight chamfer is ordinarily desired on the top face. To obtain this feature, the punch 50 is arranged so as not to flatten completely the convex face 45 of the blank, leaving a slight chamfer 55 at the corners adjacent this face.

At the completion of this operation the metal has been shaped into the blank 56 illustrated in Fig. 5-a. The corners 57 between the flats of the hexagon are completely and sharply filled out through the axial length of the blank, except for the slight chamfer 55 which is preserved on the top face of the blank. A recess 58 constituting a washer face is formed on the opposite side of the blank. Central recesses 59 and 60 are formed in the top and bottom faces, respectively, of the blank.

After the completion of the upsetting operation illustrated in Fig. 5 the punch 50 is retracted and the blank 56 is ejected from the die into the transfer mechanism by the knock-out pin 53. The blank is again turned over and transferred into alignment with a punch die 61 mounted in the bed frame 10 and illustrated in Fig. 6. The die 61 is formed with a relatively shallow opening defined by side walls 62 and an annular bottom wall 63 surrounding an axial opening 64. The walls 62 and 63 are shaped to closely fit the top face of the blank 55 and the adjacent portions of the side walls of the blank.

The punching tool is carried by the reciprocating header slide 22 and is arranged to punch an axial hole through the blank, pull the blank out of the die 61 on the retracting stroke of the punch, and then strip the blank from the punch for discharge from the machine. In the illustrated embodiment the header slide 22 is formed with a bore 65 which slidably receives a plunger 66. The plunger 66 is fixedly mounted in position in any suitable way with respect to the bed frame 10 so that it remains stationary as the header slide 22 reciprocates. The bore 65 terminates in a wall 67 which separates the bore 65 from a bore 68 extending into the slide from the front face thereof. A punch 69 is secured in position in the wall 67 and projects beyond the front face of the slide 22. A sleeve 70 is threaded or otherwise suitably secured in the bore 68 and is provided with an opening 71 slidably fitting around an inner sleeve 72. The sleeve 72 is formed with an enlarged head 73 slidably fitting in the counter-bore 74 formed in the sleeve 70. The sleeve 72 fits closely about the punch 69 and is arranged to be projected over the same to strip the blank therefrom. A plurality of rods 75 extend slidably through openings in the wall 67 and are arranged to abut at one end against the forward face of the plunger 66 and at the other end against the head 73 on the sleeve 72. The punch 69 is formed with a working end portion 76 connected to the punch by a relieved portion 77, so as to minimize friction.

When the blank 56 has been turned over and presented in alignment with the opening in the die 61 by the transfer mechanism, the punch 69 advances and enters the recess 60 in the bottom or washer face side of the blank 56. The blank 56 is first pushed into the recess in the die 61 so that its top face engages the annular bottom wall 63 and the adjacent portions of its side walls are confined by the side walls 62 of the die. The punch 69 continues to advance and shears the

wad 78 from the blank 55 to form an axial opening 79 therethrough. The punch first engages the wad 78 and starts the shearing action in the blank at a point lying in a transverse plane outside of the die 61. Thus the entire blank is permitted to swell slightly under the pressure of the punching operation, permitting free movement of the punch. Distortion of the blank is prevented, however, by the confining side walls 62 of the die 61. After the working end portion 76 of the punch has passed through the blank in the position shown in Fig. 6, the metal of the blank springs back to its initial shape, and the wad 78 is discharged through the opening 64.

As the header slide 22 is retracted the pierced blank is withdrawn from the die 61 by the working end portion 76 of the punch 69, the blank being carried on the relieved portion 77. As the header slide approaches the limit of its rearward movement the rods 75, held stationary by the plunger 66 and sliding through the wall 67, engage the head 73 of the sleeve 72 and hold the sleeve 72 stationary while the header slide and the punch 69 continue to move rearwardly. In this way the punch 69 is withdrawn into the sleeve 72, the front edge 80 of the latter engaging the pierced blank and stripping the same over the working end portion 76 of the punch 69. The finished blank 81 is then discharged from the machine and is ready for tapping.

In the preferred embodiment of this invention the blank 19 sheared from the elongated stock 8 is only slightly smaller than the opening in the die 20 so that the blank is properly guided and centered for the first blow. The opening in the die 20 is preferably cylindrical in shape with a diameter substantially equal to the diameter across the flats of the hexagonal opening in the die 28. Thus the sized blank 25 formed by the first operation is accurately guided and centered into the hexagonal opening in the die 28. The dies 33 and 46 are of substantially the same size and shape as the die 28, although a slight additional clearance may be allowed in each operation to facilitate the entry of the blank into the die. The metal displaced by the piercing noses 37 and 39 in the operation illustrated in Fig. 4 and the noses 52 and 54 in the operation illustrated in Fig. 5 flows into the blank so that the upsetting operations, in changing the external shape of the blank, need not reduce the axial height of the blank. In this way the amount of metal punched out of the blank in the wad 78 is reduced to a minimum.

The dishing operation on the blank illustrated in Fig. 4, and the subsequent flattening of the dished blank illustrated in Fig. 5, act as force multipliers on the metal of the blank adjacent the juncture of the side walls and bottom wall of the die openings so that the metal is caused to fill out the corners of the dies with a minimum of pressure applied to the front face of the blank by the punches. Thus accurate, well filled nut blanks are readily produced without excessive work hardening of the metal of the blank and without subjecting the tools and dies to excessive pressures. The operation of punching out the wad from one side of the blank with only the opposite side confined makes it possible to punch the blanks easily and accurately without distortion of the previously formed exterior surface and without encountering any difficulty in freeing the blank from the punching tool and die.

Although a preferred embodiment of the present process and apparatus has been disclosed in

considerable detail in the making of nuts it will be understood that the invention is not limited thereto, but may be employed in making many other kinds of polygonal articles or portions of articles. The various features of the invention may be employed in the combination and sequence disclosed, or separately, or in other combinations and sequences. Many other variations and modifications thereof can be resorted to without departing from the scope of the invention as defined in the following claims.

I claim:

1. The method of making polygonal articles comprising confining in a polygonal die opening a metal blank having end faces intersecting and substantially perpendicular to the sides thereof and upsetting said blank into concavo-convex form so as to force the metal of said blank against the polygonal wall of said die.
2. The method of making polygonal articles comprising upsetting metal stock into a blank having a rough polygonal outline and end faces intersecting and substantially perpendicular to the sides thereof, confining said blank in a polygonal die and upsetting said blank into concavo-convex form so as to force the metal of said blank against the polygonal wall of said die.
3. The method of making upset articles comprising confining in a die opening a blank having end faces intersecting and substantially perpendicular to the side edges thereof and upsetting said blank into concavo-convex form so as to force the side edges of said blank radially outward against the side wall of said die adjacent the convex face of said blank.
4. The method of making polygonal articles comprising upsetting metal stock to form a blank having a rough polygonal outline and end faces intersecting and substantially perpendicular to the sides thereof, confining said blank in a polygonal die and upsetting said blank into concavo-convex form so as to force the metal of said blank radially outward against the polygonal wall of said die adjacent the convex face of said blank.
5. The method of making upset articles comprising confining in a die opening a blank having end faces intersecting and substantially perpendicular to the side edges thereof and upsetting and dishing said blank into concavo-convex form so as to force the side edges of said blank radially outward against the side wall of said die adjacent the convex face of said blank.
6. The method of making polygonal articles comprising upsetting metal stock into a blank having a rough polygonal outline and end faces intersecting and substantially perpendicular to the sides thereof, and upsetting and dishing said blank into concavo-convex form so as to force the metal of said blank radially outward against the polygonal wall of the die adjacent the convex face of said blank.
7. The method of making polygonal metal articles comprising upsetting stock to form a blank having a rough polygonal outline and end faces intersecting and substantially perpendicular to the sides thereof, confining said blank in a polygonal die having a bottom wall disposed at an obtuse angle to its side walls, and upsetting the blank with a punch having a face portion substantially complementary to said bottom wall.
8. The method of making polygonal articles comprising shearing off a length of substantially cylindrical elongated stock, upsetting the sheared-off length of stock to form a concavo-convex blank having a rough polygonal outline,

confining said blank in a polygonal die and applying axial pressure to the central portion of the convex face and the peripheral portion of the concave face to flatten the convex face and force the metal of the blank radially outward against the wall of said die.

9. The method of making polygonal articles comprising shearing off a length of substantially cylindrical elongated stock, upsetting the sheared-off length of stock to form a concavo-convex blank having a rough polygonal outline, confining said blank in a polygonal die and upsetting and bending said blank in a direction to flatten the convex face thereof to force the metal of the blank radially outward against the wall of said die.

10. The method of making polygonal articles comprising shearing off a length of substantially cylindrical elongated stock, upsetting the sheared-off length of stock to form a concavo-convex blank having a rough polygonal outline, confining said blank in a polygonal die and upsetting and flattening said blank to remove the concavo-convex shape thereof and force the metal of the blank radially outward against the wall of said die adjacent the initially concave face of said blank.

11. The method of making metal articles comprising confining a blank in a die opening, upsetting said blank by axial pressure into concavo-convex form so as to force the metal of said blank radially outward against the side wall of said die adjacent the face of said blank which becomes convex, and flattening said blank in a die opening to force the metal of said blank radially outward against the side wall of said die adjacent the opposite face of said blank.

12. The method of making polygonal articles comprising confining a blank in a polygonal die opening, upsetting and dishing said blank into concavo-convex form so as to force the metal of said blank radially outward against the polygonal wall of said die adjacent the face of said blank which becomes convex, and upsetting and flattening said blank in a polygonal die opening to remove the concavo-convex form thereof and force the metal of said blank radially outward against the polygonal wall of said die adjacent the opposite face of said blank.

13. The method of making polygonal articles comprising upsetting stock to form a blank having a rough polygonal outline, confining said blank in a polygonal die opening, upsetting said blank into concavo-convex form so as to force the metal of said blank radially outward against the polygonal wall of said die adjacent the face of said blank which becomes convex, and flattening said blank in a polygonal die opening to force the metal of said blank radially outward against the polygonal wall of said die adjacent the opposite face of said blank.

14. The method of making polygonal articles comprising upsetting stock to form a blank having a rough polygonal outline, confining said blank in a polygonal die opening, upsetting and bending said blank into concavo-convex form so as to force the metal of said blank radially outward against the polygonal wall of said die adjacent the face of said blank which becomes convex, and thereafter flattening said blank in a polygonal die opening to remove the concavo-convex form thereof and force the metal of said blank radially outward against the polygonal wall of said die adjacent the opposite face of said blank.

15. The method of making polygonal articles comprising upsetting stock to form a polygonal blank having a rough polygonal outline in section and end faces substantially perpendicular to its side walls, confining said blank in a polygonal die opening, upsetting and bending said blank into concavo-convex form so as to force the metal of said blank radially outward against the polygonal wall of said die adjacent the face of said blank which becomes convex, and flattening said blank in a polygonal die opening to remove the concavo-convex form thereof and force the metal of said blank radially outward against the polygonal wall of said die adjacent the opposite face of said blank.

16. The method of making nuts and the like comprising confining a blank in a polygonal die having a bottom wall disposed at an angle to its side walls different than the angle between the corresponding portions of the blank, upsetting the blank by pressing the same with a punch having a face portion substantially complementary to said bottom wall, removing the blank from said die, and thereafter punching an axial hole through said blank.

17. The method of making nuts and the like comprising confining in the side walls of a polygonal die, the side edges of a blank having a concavo-convex shape, upsetting and bending said blank to flatten the concave face thereof and force the metal of the blank radially outward against the wall of said die, removing the blank from said die, and thereafter punching an axial hole through said blank.

18. The method of making nuts and the like comprising confining a blank in a polygonal die opening, upsetting said blank into concavo-convex form so as to force the metal of said blank radially outward against the polygonal wall of said die adjacent the face of said blank which becomes convex, flattening said blank in a polygonal die opening to force the metal of said blank radially outward against the polygonal wall of said die adjacent the opposite face of said blank, and thereafter punching an axial hole through said blank.

19. The method of making nuts and the like comprising upsetting stock to form a blank having a rough polygonal outline, confining said blank in a polygonal die opening, upsetting said blank into concavo-convex form so as to force the metal of said blank radially outward against the polygonal wall of said die adjacent the face of said blank which becomes convex, flattening said blank in a polygonal die opening to force the metal of said blank radially outward against the polygonal wall of said die adjacent the opposite face of said blank, and thereafter punching an axial hole through said blank.

20. The method of making nuts and the like comprising upsetting stock to form a polygonal blank having a rough polygonal outline in section and end faces substantially perpendicular to its side walls, confining said blank in a polygonal die opening, upsetting and bending said blank into concavo-convex form so as to force the metal of said blank radially outward against the polygonal wall of said die adjacent the face of said blank which becomes convex, flattening said blank in a polygonal die opening to remove the concavo-convex form thereof and force the metal of said blank radially outward against the polygonal wall of said die adjacent the opposite face of said blank, and thereafter punching an axial hole through said blank.

## 11

21. The method of making metal articles comprising forming a blank having a side wall and end faces intersecting said side wall at peripheral corners, confining the side wall of the blank in a die opening, applying axial pressure to said blank by tool and die surfaces initially engaging the same at the central portion only of one end face and adjacent the peripheral corner only of the opposite end face, and bending and upsetting the blank by such pressure about neutral axes within the axial length of the blank to bring the end faces into substantially full engagement with said tool and die surfaces without punching through the blank.

22. The method of making polygonal articles comprising upsetting a piece of metal into a blank having a side wall substantially polygonal in cross-section and end faces intersecting said side wall at substantially polygonal corners, confining the side wall of said blank in a polygonal die opening, applying axial pressure to said blank by tool and die surfaces substantially co-extensive with said end faces and initially engaging the blank at the center of one end face and adjacent the polygonal corner of the opposite end face while leaving the polygonal corner of the said one end face free to move radially inward and the center of said opposite end face free to move axially, and bending and upsetting the blank by such pressure about neutral axes within the axial length of the blank to bring the end faces into substantially full engagement with said tool and die surfaces and force the polygonal corner of said opposite end face radially against the die.

23. The method of making metal articles comprising forming a blank having a side wall and end faces, one of said end faces being concave, confining said blank in a die having a side wall and a bottom wall with the peripheral portion of the concave end face of said blank engaging the bottom wall of said die and the central portion of said concave end face spaced from said bottom wall, and with the side wall of said blank engaging the side wall of said die adjacent said bottom wall, applying axial pressure to the central portion of the opposite end face of said blank and bending the blank by such pressure to bring said one end face into full engagement with the bottom wall of said die, thereby increasing the length of the peripheral portion of said concave end face and pressing the same against the die.

24. The method of making polygonal articles comprising shearing off a length of substantially cylindrical elongated stock, upsetting the sheared off length to form a metal blank having a polygonal side wall and end faces, one of said end faces being concave, confining the side wall of said blank in a polygonal die opening, applying axial pressure to said blank by tool and die surfaces initially engaging the blank at the peripheral portion only of the concave end face and the central portion only of the opposite end face, and bending the blank by such pressure to flatten said concave face and force the peripheral portion thereof radially against the die.

25. The method of making nuts and the like comprising forming a metal blank having a side wall and end faces, confining said blank in a polygonal die having a bottom wall engaging the peripheral portion of one end face of the blank and spaced from the central portion thereof, applying axial pressure to the opposite end face of said blank to bend the blank into full engage-

## 12

ment with said bottom wall, removing the blank from said die, turning the blank over and confining the same in a second polygonal die having a bottom wall engaging the peripheral portion of said opposite end face of the blank and spaced from the central portion thereof, and applying axial pressure to the blank to bend the same into full engagement with the bottom wall of said second die.

26. The method of making upset articles comprising shearing off a length of elongated stock, upsetting the sheared off length into a blank having concavo-convex end faces and a peripheral side wall, confining the side wall of the blank in the side wall of a die with the concave end face of the blank having its peripheral portion engaging the bottom wall of the die and its central portion spaced therefrom, and upsetting and flattening said blank by axial pressure to force the metal of the blank radially outward against the side wall of the die.

27. The method of making polygonal articles comprising shearing off a length of substantially cylindrical elongated stock, forging the sheared off length into a blank having end faces and a side wall of rough polygonal shape, one of said end faces having an axial recess extending into but not entirely through said blank, said one end face including a concave portion radially outside of said recess, confining said blank in a die opening having a polygonal side wall, engaging said one end face with a die surface having an annular flat portion forming sharp right-angled corners with the polygonal side wall of said die opening, said flat portion initially engaging said one end face of said blank adjacent the periphery thereof with the remainder of said die surface spaced axially from said one end face, pressing said blank axially against said die surface, and flowing the metal of said blank by such pressure into full engagement with said annular flat portion and with the sharp corners formed by said annular flat portion and the polygonal side wall of said die opening.

28. The method of making polygonal articles comprising shearing off a length of substantially cylindrical elongated stock, forging the sheared off length into a blank having end faces and a side wall of rough polygonal shape, one of said end faces having an axial recess extending into said blank, said one end face including a concave portion radially outside of said recess, confining said blank in a die opening having a polygonal side wall, engaging said one end face with a die surface having one annular flat portion forming sharp right-angled corners with the polygonal side wall of said die opening and a depressed annular flat portion radially within and parallel to said one annular flat portion and spaced axially therefrom by a substantially cylindrical shoulder, said one flat portion initially engaging said one end face of said blank adjacent the periphery thereof with the remainder of said die surface spaced axially from said one end face, pressing said blank axially against said die surface, and flowing the metal of said blank by such pressure into full engagement with both said annular flat portions, said cylindrical shoulder, and the sharp corners formed by said annular flat portion and the polygonal side wall of said die opening.

29. The method of making polygonal articles comprising shearing off a length of substantially cylindrical elongated stock, forging the sheared-off length into a blank having end faces and a

side wall of rough polygonal shape, each of said end faces having an axial recess extending into but not entirely through said blank, one of said end faces including a concave portion radially outside of its recess, the opposite end face including a convex portion substantially aligned with said concave portion, confining said blank in a die opening having a polygonal side wall, engaging said one end face with a die surface having an annular flat portion forming sharp right-angled corners with the polygonal side wall of said die opening, said flat portion initially engaging said one end face of said blank adjacent the periphery thereof with the remainder of said die surface spaced axially from said one end face and pressing said blank axially against said die surface to flatten said convex portion and flow the metal of said blank into full engagement with said annular flat portion and with the sharp corners formed by said annular flat portion and the polygonal side wall of said die opening.

30. The method of making polygonal articles comprising shearing off a length of substantially cylindrical elongated stock, forging the sheared-off length into a blank having end faces and a side wall of rough polygonal shape, each of said end faces having an axial recess extending into said blank, one of said end faces including a concave portion radially outside of said recess, the opposite end face including a convex portion substantially aligned with said concave portion, confining said blank in a die opening having a polygonal side wall, engaging said one end face with a die surface having one annular flat portion perpendicular to the polygonal side wall of said die opening and abutting the same in sharp corners and a depressed annular flat portion radially within and parallel to said one annular flat portion and spaced axially therefrom, said one flat portion initially engaging said one end face of said blank adjacent the periphery thereof with the remainder of said die surface spaced axially from said one end face, pressing said blank axially against said die surface to flatten said convex portion, and flowing the metal of said blank by such pressure into full engagement with both said annular flat portions and said cylindrical shoulder and the sharp corners formed by said annular flat portion and the polygonal side wall of said die opening.

31. The process of making polygonal nuts consisting of shearing off a length of substantially cylindrical elongated stock, confining the sheared-off length in a substantially cylindrical first die and exerting pressure on the end faces thereof to size the same, confining the sized blank in

a polygonal second die and exerting pressure on the opposite end faces thereof to flow the metal of the blank into a rough polygonal outline, confining the blank so produced in a polygonal third die and exerting pressure on the opposite end faces of the blank to form axial recesses in said end faces separated by an integral web in the blank and to further shape the polygonal side wall of the blank, then confining the blank in a polygonal fourth die, pressing one end face of the blank against a die surface having one annular flat portion forming sharp right angled corners with the polygonal side wall of said fourth die and a depressed annular surface radially within said one annular surface and spaced therefrom by a substantially cylindrical shoulder, flowing the metal of the blank by such pressure in the fourth die into full engagement with said annular flat portions, said shoulder, and the corners between said one annular flat surface and the polygonal wall of said fourth die, and then confining the blank in a polygonal fifth die and punching an axial hole therethrough.

JOHN H. FRIEDMAN.

25

#### REFERENCES CITED

The following references are of record in the file of this patent:

#### UNITED STATES PATENTS

|    | Number    | Name          | Date           |
|----|-----------|---------------|----------------|
| 30 | 680,991   | Crosby        | Aug. 20, 1901  |
|    | 808,177   | Thiem         | Dec. 26, 1905  |
|    | 965,039   | Slick         | July 19, 1910  |
| 35 | 1,342,676 | Hollings      | June 8, 1920   |
|    | 1,730,377 | Northrup      | Oct. 8, 1929   |
|    | 1,795,518 | Sharp         | Mar. 10, 1931  |
|    | 1,837,720 | Luce et al.   | Dec. 22, 1931  |
|    | 1,946,618 | Fitch et al.  | Feb. 13, 1934  |
| 40 | 1,977,162 | Wilcox        | Oct. 16, 1934  |
|    | 1,993,137 | Gibney        | Mar. 5, 1935   |
|    | 2,015,596 | Harvey        | Sept. 24, 1935 |
|    | 2,016,296 | Rosborough    | Oct. 8, 1935   |
|    | 2,057,527 | Johnson       | Oct. 13, 1936  |
| 45 | 2,170,473 | Fitch         | Aug. 22, 1939  |
|    | 2,207,391 | Wilcox        | July 9, 1940   |
|    | 2,226,399 | Frayer        | Dec. 24, 1940  |
|    | 2,287,214 | Wilcox        | June 23, 1942  |
|    | 2,352,265 | Kapple et al. | June 27, 1944  |
| 50 | 2,393,850 | Wilcox        | Jan. 29, 1946  |

#### FOREIGN PATENTS

|    | Number  | Country       | Date          |
|----|---------|---------------|---------------|
| 55 | 216,401 | Germany       | Nov. 13, 1919 |
|    | 304,122 | Germany       | Mar. 4, 1918  |
|    | 5,916   | Great Britain | Mar. 9, 1912  |